

## UNITED STATES PATENT OFFICE

2,691,588

PHOTOGRAPHIC DEVELOPERS CONTAINING  
8-HYDROXYQUINOLINES

Richard W. Henn and John I. Crabtree, Rochester, N. Y., assignors to Eastman Kodak Company, Rochester, N. Y., a corporation of New Jersey

No Drawing. Application March 14, 1952,  
Serial No. 276,676

4 Claims. (Cl. 95—88)

1

This invention relates to photography and particularly to photographic developers having reduced tendency to oxidation caused by heavy metals.

Fog in photographic emulsions is produced in several ways, one of which is the rapid oxidation of the developer when the emulsion is exposed to the air while wet with developer. Fog of this type which is known as aerial fog occurs chiefly in the presence of oxidizing catalysts such as ions of copper and ferric iron (Dundon and Crabtree, Transactions of the Society of Motion Picture Engineers, vol. 12, page 1096; American Photography, December 1924, page 742). Significant amounts of copper are of the order of  $10^{-9}$  to  $10^{-6}$  mole per liter. These amounts are likely to be present in commercial grades of chemicals used for photographic developers.

Numerous materials have been suggested to prevent this type of fog, these materials forming extremely insoluble or undissociated compounds of iron, copper, or other heavy metals. Materials such as cyanides, sulfides, a number of organic complex formers, desensitizers such as pinakrytol green and phenoxyfranin have been suggested but these compounds either produce stain or are otherwise unsatisfactory.

It is therefore an object of the present invention to provide photographic developers which are not subject to the formation of fog produced by heavy metals in the solution. Another object is to provide photographic developers having reduced tendency to oxidation caused by heavy metals such as iron and copper. A still further object is to provide color forming photographic developers which are not subject to the oxidizing action of heavy metals.

These objects are accomplished by incorporating in the developing solution an 8-hydroxyquinoline especially an 8-hydroxyquinoline-5-sulfonic acid.

The developing solutions which we propose to use contain a silver halide developing agent such as paraphenylene diamine, diethyl paraphenylene diamine, 2-amino-5-diethylaminotoluene, hydroquinone, N-methyl para-aminophenol, an alkali metal sulfite such as sodium or potassium sulfite or equivalent material such as potassium bisulfite, and an 8-hydroxyquinoline. Among the 8-hydroxyquinolines which may be used for this purpose are 8-hydroxyquinoline-5-sulfonic acid, 7-chloro-8-hydroxyquinoline-5-sulfonic acid, 7-bromo-8-hydroxyquinoline-5-sulfonic acid, 7-methyl-8-hydroxyquinoline-5-sulfonic acid and 6-methyl-8-hydroxyquinoline-5-sulfonic acid. The developing solution is an alkaline solution

containing a suitable alkaline material such as sodium carbonate, sodium hydroxide or sodium metaborate. Other customary developer ingredients may also be present.

The following examples illustrate developer formulas constituted according to our invention.

## Example I

|    |                                                 | Grams |
|----|-------------------------------------------------|-------|
| 10 | Sodium metaborate                               | 1.0   |
|    | Sodium sulfite (anhyd.)                         | 4.0   |
| 15 | 2-amino-5-diethylaminotoluene monohydrochloride | 3.0   |
|    | Sodium carbonate (mono.)                        | 20.0  |
|    | Potassium bromide                               | 2.0   |
|    | 8-hydroxyquinoline-5-sulfonic acid              | 0.25  |
|    | Water to 1 liter.                               |       |

## Example II

|    |                                    | Grams |
|----|------------------------------------|-------|
| 20 | Elon                               | 5.0   |
|    | Sodium sulfite                     | 100.0 |
|    | Sodium carbonate                   | 2.5   |
| 25 | Ethylenediamine sulfate            | 12.0  |
|    | 8-hydroxyquinoline-5-sulfonic acid | 0.25  |
|    | Water to 1 liter.                  |       |

## Example III

|    |                                 | Grams |
|----|---------------------------------|-------|
| 30 | Hydroquinone                    | 2.5   |
|    | Elon                            | 5.0   |
|    | Sodium sulfite                  | 100.0 |
| 35 | Sodium metaborate               | 20.0  |
|    | Ethylenediamine tetracetic acid | 5.0   |
|    | 8-hydroxyquinoline-sulfate      | 1.0   |
|    | Water to 1 liter.               |       |

The 8-hydroxyquinolines may be present in the developer in amounts varying from about 0.05 gram to about 2.5 grams per liter of developing solution. The exact quantity to be used will depend on the concentration of the metal ion to be sequestered.

Developers containing primary aliphatic amines such as guanidine, ethanolamine, ethylenediamine, morpholine or other chelating compounds such as triglycine are especially subject to bad catalytic oxidation in the presence of heavy metals. Examples II and III illustrate such developers. In the case of Example II, the addition of two parts of copper per million to the developer without the 8-hydroxyquinoline-5-sulfonic acid decreased the aeration life to a stream of finely divided air bubbles from 24 to 6 hours. When the 8-hydroxyquinoline-5-sulfonic acid was added the aeration life was restored to its normal of 24 hours. A similar effect was observed in the case of Example III.

## 3

The color developer of Example I shows especially good aeration life and is used for developing an emulsion containing color couplers, for example, for developing a film such as that described in Jelley and Vittum U. S. Patent 2,322,027.

In certain cases, the 8-hydroxyquinolines of our invention may be incorporated in the emulsion, overcoat, backing layer or interlayer of a film.

It will be understood that the examples and modifications included herein are illustrative only and that our invention is to be taken as limited only by the scope of the appended claims.

What we claim is:

1. A photographic developing solution having reduced tendency to oxidation caused by heavy metals and capable of forming a colored image upon development of an exposed silver halide emulsion in the presence of a color coupler, comprising an alkaline solution of a primary aromatic paradiamino developing agent, an alkali metal sulfite, and 8-hydroxyquinoline-5-sulfonic acid.

2. A photographic developing solution having reduced tendency to oxidation caused by heavy metals and capable of forming a colored image upon development of an exposed silver halide emulsion in the presence of a color coupler, comprising an alkaline solution of 2-amino-5-diethylaminotoluene, sodium sulfite, and 8-hydroxy- 30

## 4

3. A photographic developing solution having reduced tendency to oxidation caused by heavy metals and capable of forming a colored image upon development of an exposed silver halide emulsion in the presence of a color coupler, comprising an aqueous solution of sodium carbonate, 2-amino-5-diethylaminotoluene, sodium sulfite and approximately 0.25 gram per liter of solution of 8-hydroxyquinoline-5-sulfonic acid.

4. A photographic developer having reduced tendency to oxidation caused by heavy metals, comprising an alkaline solution of a silver halide developing agent, an alkali metal sulfite, an aliphatic amine, and a compound selected from the class consisting of 8-hydroxyquinoline, 8-hydroxyquinoline-5-sulfonic acid and 8-hydroxyquinoline-5-sulfonic acid substituted with a member of the class consisting of halogen and alkyl.

## 20 References Cited in the file of this patent

## UNITED STATES PATENTS

| Number    | Name           | Date          |
|-----------|----------------|---------------|
| 2,168,181 | Ulrich et al.  | Aug. 1, 1939  |
| 2,268,419 | Paul           | Dec. 30, 1941 |
| 2,381,863 | Benignus       | Aug. 14, 1945 |
| 2,524,741 | Tulagin et al. | Oct. 3, 1950  |
| 2,544,649 | Bersworth      | Mar. 13, 1951 |
| 2,596,978 | Burtner        | May 20, 1952  |